

## UNITED STATES PATENT OFFICE.

OTTO MATTHIES, OF DESSAU, PETER WULFF, OF STARNBERG, AND WALTER DIETELE AND BRUNO WENDT, OF DESSAU, GERMANY, ASSIGNORS TO I. G. FARBENINDUSTRIE AKTIENGESELLSCHAFT, OF FRANKFORT, GERMANY.

PROCESS OF MANUFACTURING PHOTOGRAPHIC SILVER HALIDE EMULSIONS AND PRODUCTS OBTAINED THEREBY.

No Drawing. Application filed July 10, 1926, Serial No. 121,731, and in Germany July 25, 1925.

It is known that sulphydric acid or sulphides produce more or less fog in photographic silver halide emulsions. Although attempts have been made to add only very 5 minute, exactly defined, quantities of these chemical compositions, they generally are found to produce fog, although a certain increase in the sensitivity of the emulsion may be perceived at the same time.

10 The sensitivity of photographic silver halide emulsions may be raised without fogging, according to the present invention, by adding to the emulsion, during emulsion making, small quantities of salts soluble in water, the anions of which contain at least 15 three atoms of sulphur. The addition may be made to the constituents of the emulsion, or at any step of emulsion making, or to the finished emulsion.

20 The compounds adapted to be added for this purpose, e. g. sodium trithionate, sodium tetrathionate, the sodium salt of the trithio-di-glycolic acid

25 (COOH.CH<sub>2</sub>.S.S.S.CH<sub>2</sub>.COOH), produce the desired effect in emulsions having an alkaline reaction, as well as in neutral and weakly acid emulsions. With silver-ions they form silver-compositions which 30 are difficultly soluble in water and decompose spontaneously producing a silver-metallocid-composition.

The decomposable silver-sulphur-compounds having been formed in the silver 35 halide crystals formerly free from sulphur, or on their surfaces, the decomposition producing silver-metallocid takes place in the emulsion. The invention depends on the knowledge that the sensitivity of photographic emulsions is raised in a particularly 40 good manner when traces of silver-metallocid, especially of silver sulphide,—constituting reducing agents,—are produced by the decomposition of the above-mentioned decomposable compounds inside of the silver halide 45 crystals or on their surfaces. The use of soluble sulphides or of colloidal silver sulphide solutions never results in analogous increases in the sensitivity of the halide 50 emulsions.

Selenium and tellurium are equivalent to

sulphur in the compositions adapted for this purpose.

The process described makes it possible to produce emulsions of high sensitivity with 55 gelatines heretofore thought to be photographically unsuitable, since up to now only a few gelatines produced in the manufacture of gelatine could be used, and the selection of the operable gelatines involved great 60 trouble and expense. By the process according to the present invention the manufacture of photographic emulsions becomes much more reliable than previously and the sensitivity of the emulsions markedly may 65 be raised.

*Example 1.*

To a photographic silver halide emulsion prepared from 1 kg. of gelatine and 400 g. of silver nitrate, there is added 50-100 mg. of 70 sodium trithionate. By this addition the sensitivity increases from 12° to 17° Scheiner.

*Example 2.*

75 The same effect is reached by substituting for the sodium trithionate in Example 1, 30-40 mg. of the sodium salt of the trithio-di-glycolic acid.

*Example 3.*

To the emulsion manufactured according to Example 1, there is added, instead of sodium trithionate, 5 ccm. of a *n*/10 solution of potassium selenotrichionate which is obtained by dissolving selenium in potassium sulphite.

Having now particularly described and ascertained the nature of our invention and in what manner it is to be performed, we 90 declare that what we claim is:

1. Process of making a photographic silver halide emulsion which comprises incorporating in said emulsion a water-soluble salt the anions of which contain at least 95 three atoms of an element of the sulphur group.

2. Process of manufacturing photographic silver halide emulsions which comprises adding to the emulsion water-soluble salts the 100 anions of which contain at least three atoms of an element of the sulphur group.

3. Process of manufacturing photographic silver halide emulsions which comprises adding to the emulsion water-soluble salts the anions of which contain at least three atoms of sulphur. 15
4. Silver halide emulsions comprising a colloid, particles of silver halide suspended therein, and added water-soluble compounds the anions of which contain at least three 10 atoms of an element of the sulphur group.
5. Photographic layers comprising silver halide emulsions as defined in claim 4.
6. A silver halide emulsion comprising gelatine, particles of silver halide suspended therein, and a small amount of a water-soluble compound the anions of which contain at least three atoms of sulphur. 15
7. Photographic layers comprising the silver halide emulsion defined in claim 6. 20
- In testimony whereof we affix our signatures.

OTTO MATTHIES.  
WALTER DIETERLE.  
PETER WULFF.  
BRUNO WENDT.